# EUROPEAN PATENT SPECIFICATION

(11) **EP 0 114 000 B1**
(45) Date of publication and mention of the grant of the patent: **01.10.1986**
(21) Application number: 83307923.9
(22) Date of filing: 22.12.1983
(51) Int. Cl.: H01B 3/00, H05K 7/20

(54) **Thermally conducting filler for enclosing electrical components**
Wärmeleitende Füllmasse zum Einkapseln elektrischer Bauteile
Charge thermoconductrice pour capsuler des composants électriques

(30) Priority: 11.01.1983 US 457199
(43) Date of publication of application: 25.07.1984
(73) Proprietor: Ferranti plc, Cheadle Cheshire SK8 4HZ (GB)
(72) Inventor: Lien, Charles, Huntington New York 11743 (US); Whitehead, Derek Wayne, Locust Valley New York 11560 (US)
(74) Representative: Bradley, David Nicholas

## Description

### Background of the Invention

This invention relates to a novel fhermally conductive filler for insulating the interior of a housing containing electrical components and to a method of filling the housing and encapsulating the electrical components with the thermally conductive medium.

It is well known that heat produced by electrical components contained within a housing should be removed by conducting the heat to the exterior of the housing. When the electrical components within the housing are relatively high voltage components and the housing has a relatively small volume, it is not feasible to employ conventional air cooling or liquid cooling systems. Moreover, it is frequently desirable that the housing be filled with a medium which will encapsulate and protect the individual components therein against relative movement due to shock forces and the like, and against chemical attack or contamination by environment influences. Consequently, electrical equipment including such assemblies as high voltage power supplies which produce output voltages of the order of thousands of volts, are conventionally potted by a potting material which is typically a polymerized resin.

These potting resins provide mechanical protection of the potted components but the thermal conductivity of such resins is relatively poor. For example, the thermal conductivity of typical potting material now used is of the order of 0.00021 kW/m.k (0.0005 cal/sec.cm.°C). Therefore, heat generated by the electrical components within the housing is not easily conducted to external surfaces of the housing.

It is known that thermally conductive particles can be added to polymerized potting resins in order to increase the thermal conductivity of the potting material. These thermally conductive particles are generally electrically insulative ceramics which have good thermal conduction characteristics and typically may be beryllium oxide, aluminium oxide, boron nitride or some types of silicon carbide. These thermally conductive particles are normally stirred into the potting resin just before the resin is poured into the interior of a housing.

U.S. patent 4,265,775, for example, describes the use of a number of these thermally conductive materials in particle or powder form, whilst U.S. patent 3,137,665 refers to the use of granular inorganic fillers of the same type. British patent No. 874,801 describes the use of crystalline silicon carbide as a filler, though this is not an electrically-insulating material. German patent 1,439,456 describes the use of a material which includes fine particles of, for example, quartz, metal, metal oxide or metal carbide to improve heat dispersal.

It has been found that the volume of the insulation particles loaded in this way can rarely exceed 50% of the total resin volume. Consequently, the thermal conductivity of the insulation medium with the added particles is usually only about twice that of the resin itself. Thus, while aluminium oxide, for example, has a bulk thermal conductivity of 0.035 kW/m.K (0.084 cal/sec.cm °C) when particles of the ceramic consists of about 50% of the total volume of a conventional polymerized potting resin, the thermal conductivity of the ultimate material will be increased from about 0.00021 kW/m.K (0.0005 cal/sec.cm °C) to about 0.00042 kW/ m.K (0.001 cal/sec.cm °C).

### Brief Description of the Invention

In accordance with the invention, the interior of an electrical housing filled with heat-generating devices, such as transistors, transformers, resistors and the like, having irregular volumes and shapes, is filled with and easily flowing slurry consisting of a mixture of more than 50% by volume and preferably more than 70% by volume of heat-conductive, electrically insulative particles, suspended in a dielectric fluid, together with a plurality of freely-suspended filler blocks of a material having the same properties as the mixture. The dielectric fluid is preferably a liquid such as silicone oil. The thermally conductive particles typically may be aluminium oxide particles or the like having a particle size which is preferably distributed about a mean diameter of about 150 micrometer. Beryllia can also be used, but it is more expensive than aluminum and is very toxic in powdered form.

The filler blocks may be of any required size and shape, since their purpose is simply to reduce the quantity of the slurry required to fill a space. The term "freely-suspended" as used with reference to the filler blocks means that they are not attached to the housing or to any of the components contained therein and are substantially surrounded by the slurry.

The slurry is first mixed at room temperature by pouring the particles into the dielectric fluid and agitating this mixture. Slurry is then poured into a filler column which, in turn, is connected to the open top of the electrical housing. As the level of the slurry reaches large empty spaces in the housing solid filler blocks of appropriate size are fed into the housing, followed by more slurry. The filler column and housing are sealed to be air-tight so that the slurry cannot freely escape from the interior of the housing. The slurry is then subjected to vacuum to remove trapped air bubbles therefrom and the slurry is permitted to settle into the housing interior under the force of gravity. During the settling period, the assembly is tilted in different directions to eliminate Rankine slope effects. Oil appearing at the top of the column is decanted and replaced by additional slurry during the settling process. The volumetric packing density after settling for about 36 hours will often exceed 80% of particles by volume.

The slurry particles and filler blocks are then further compacted against one another to form a relatively non-flowable paste. This further compacting can be carried out by a centrifugal process. Thus, the entire housing is spun at moderate 'g" force for about two hours in a suitable fixture. The insulation particles and filler blocks, which are more dense than the suspending liquid, tend to compact in one direction relative to the housing due to centrifugal force effects and the particles form a paste-like consistency in which silicone oil fills the interstices between particles. The paste now forms an almost solid continuous body which encapsulates the components and extends between the components and to the interior of the surrounding walls of the housing. It has been found that the final highly compacted mass has a thermal conductivity close to that of a solid block of the insulation material which is employed.

The filler column is then removed and the paste, which extends above the top of the open housing end, is sliced off to be flush with the housing top. A housing lid is then sealed over the housing top to complete the enclosure.

Preferably, the housing is made of conductive material to act as a heat sink to heat conducted form internal potted components through the encapsulant.

### Brief Description of the Drawings

Figure 1 is a cross-section taken through a housing which has been filled with thermally conductive insulation in accordance with the invention.
Figure 2 is a cross-section view of Figure 1 taken across the section line 2-2 in Figure 1.

### Detailed Description of the Drawings

Referring to the drawings, there is shown in generalized form a housing 10 which may be of a good thermal conductor, preferably of aluminium, and which may have any desired thickness. Housing 10 has a top lid 11 attached and sealed thereto in any desired manner. The housing 10 can typically have dimensions of 5 cm (2 inches) by 10 cm (4 inches) by 12.5 cm (5 inches) but it will be obvious that the invention can apply to any housing size which contains any type of component.

Various heat-generating electrical components are mounted within the housing and are schematically illustrated as the heat-generating components 12, 14, 16, 18, 20 and 22. These components can be of any desired nature. By way of example, component 12 could be a bridge-connected rectified circuit which might produce 4.8 watts during its operation. Component 14 could be an inverter transformer which produces 25 watts during its operation. Components 16 to 22 could be the elements of a bridge-connected rectifier which produces 1.2 watts. Components 16 to 22 can be carried on a common circuit board with other components, not shown. An electrical connector shown in the form of a multi-conductor ribbon 24 carries suitable wires from the interior electrical components of housing 10 to the exterior where the wires can be connected to other circuits. A suitable insulation seal can enclose and seal ribbon 24 as it passes through the wall of housing 10. Alternatively, a multi-pin connector can be formed in the wall of housing 10 and individual wires from the components within housing 10 can be connected to the multi-pin connector.

In order to prevent an excessive temperature rise of components 16 to 22 and their connecting leads or wires during their operation without complicating the housing design with metal heat sinks, and without having to enlarge the housing, the components can be thermally connected to the exterior walls of housing 10 by the noval heat conductive insulation of the invention which encapsulates the electrical components.

The housing 10 is provided with an open top (lid 11 is removed) and the electrical components to be mounted therein are fixed in place. A filler column (not shown) which has a volume larger than that of housing 10, is sealed to the top of housing 10.

In accordance with the invention, an insulation medium is prepared as a relatively non-viscous slurry of particles of a material having good thermal conductive properties but which are electrically insulative, suspended in an insulation fluid. Typical particles may be of aluminium oxide, beryllium oxide, boron nitride and certain types of known silicon carbides. The particle size employed for these particles is not critical. Good results have been obtained with particles distributed about a mean diameter of less than about 300 micrometer which ensures uniform and homogeneous filling of the particles within housing 10 and into very small irregular crevices or the like, in the interior of housing 10.

The particles are loaded into a suitable dielectric fluid as silicone oil at room temperature an stirred to ensure thorough mixing and uniform distribution of the particles into the oil. There should be sufficient oil present in the mixture to ensure that the slurry will flow easily into the interior of housing 10. The particles should occupy more than one half by volume of the slurry.

In an illustrative embodiment of the invention, aluminium oxide particles have a size distributed around a mean diameter of about 150 micrometer are stirred into a silicone oil carrier. The powder and oil are in a ratio of about 70% to 30% respectively, by volume. The slurry is very easily flowable in this condition. Other stable dielectric fluids can be used in place of silicone oil.

The slurry is then poured into the filler column connected to container 10 of Figure 1 and 2. When the interior of the housing contains large voids solid filler blocks, such as blocks 34 and 36, are added, followed by further quantities of the slurry, and this is repeated until the container is full. Further slurry is added to at least partially fill the filler column. A vacuum is then applied to the filler column and housing to remove trapped air bubbles and the slurry is then permitted to settle into container 10 for a given settling period, for example, 36 hours. During this settling period, the unit an column are tilted to different orientations to eliminate Rankine slope effects. During the settling period, oil at the top of the column is decanted and is replaced with the 70% to 30% by volume slurry.

At the end of the settling period, the alumina particles will reach a packing density in excess of 80% by volume of the slurry.

The assembly is then placed in a centrifugal apparatus and is rotated at a moderate "g" force to cause the aluminium oxide particles to compact further. The compacted particles and filler blocks now form an almost solid past-like body which adheres to all exposed surfaces within housing 10 and which encapsulates all components within the housing.

Thereafter, excess silicone fluid is drawn off from the top of the column and the column is removed. The paste, which extends above the top of container 10, is sliced through at the column to container joint.

A conductive lid 30 is then fastened to the top of housing 10. A compressible synthetic rubber pad 31 is fixed to the interior of lid 31 to keep the paste under positive pressure within housing 10.

Paste compacted in this way and employing aluminium oxide particles had a thermal conductivity of the order of 0.0293 kW/m.K (0.07 cal/sec.cm °C) as compared with a thermal conductivity of 0.035 kW/m.K (0.084 cal/sec.cm °C) for the solid material.

Afterfilling, small cavities may appear within the paste as a result of thermal movement. These cavities are not important to thermal behaviours, but they could be significant in terms of formation of corona discharge. However, oil in and around the alumina will fill these cavities as they form to prevent electrical breakdown within the cavities.

The blocks can have any desired shape and reduce the volume of compacted particles needed to fill the housing interior. The filler blocks 34 and 36 may be of the same ceramic material as the particles of the slurry and, in the preferred example, are of aluminium oxide.

In a specific example of the invention, the electrical components 12 through 22 were capable of having a working surface temperature of 220°C. The mean free path distances from the surfaces of components 12 and 14 and of components 16,18,20 and 22 collectively was 25 mm (1 inch), 10 mm (0.375 inch) and 25 mm (1 inch) respectively, and their effective areas were 13 square cm (2 square inches), 255 square cm (8 square inches) and 26 square cm (4 square inches) repectively. The thermally conductive paste encapsulated and coupled these components to the surfaces of housing 10 so that the housing 10 had a temperature of about 210°C., indicating a temperature differential across the thermally conductive insulating material of only 10°C.

In another example, a magnetic/rectifier module of a 550 watt inverter, working at 1 watt per cubic cm (16 watts per cubic inch) had an internal dissipation of the order of 30 watts. The steady state temperature difference between the centre module and the outside walls was less than five centigrade degrees.

It is important to examine the variation of thermal conductivity for the encapsulating material with the proportion of filler. This is tabulated in the following table for two theoretical materials, one a thermally condutive powder and one a fluid. The thermal conductivities are shown for three alternative thermal conductivity ratios of the powder to fluid of 10:1, 100:1, 1000:1.

It is seen that for proportions of the higher thermal conductivity material, up to about 70% by volume, there is no significant difference in the achieved thermal conductivity, irrespective of whether the conductivity ratios are 10:1, 100:1, or 1000:1. This result covers the range of proportions which can be obtained with loaded encapsulating resins (due to limitations in pour and infill), and shows the restriction imposed by the resin itself.

The table also shows that it would be valuable to achieve volumatic fill proportions of the more conductive material of greater than about 80%, and specifically in the range from 90% to 96%, and thereby obtain a significant proportion of the available benefits of the material with a ratio of 100:1. The table also shows that the benefits of a 1000:1 material cannot be obtained until a loading of virtually 100% has been achieved.

Although a preferred embodiment of this invention has been decribed, many variations and modifications will now be apparent to those skilled in the art, and it is therefore preferred that the instant invention be limited not be the specific disclosure herein, but only by the appending claims.

## Claims

1. A thermally-conducting filler for enclosing electrical components contained in a housing, the filler comprising a mixture of electrically-insulating thermally-conducting particles and a dielectric fluid forming a slurry which is adapted to completely and homogeneously fill any spaces in said housing, the particles comprising greater than about 50% by volume of the slurry prior to being introduced into the housing and being capable of being subsequently compacted to form a paste in which the particles comprise greater than 80% by volume, characterised in that the filler includes a plurality of freely-suspended filler blocks of a material having the same properties as the said mixture so as to reduce the volume of said mixture required to fill the housing.

2. A filler as claimed in Claim 1 characterised in that said particles have a mean diameter of about 150 micrometer.

3. A filler as claimed in either of Claims 1 or 2 characterised in that the particles are formed from a ceramic material.

4. A filler as claimed in Claim 3 characterised in that the ceramic material is selected from the group comprising metal oxides, metal nitrides and metal carbides.

5. A filler as claimed in anyone of Claims 1 to 4 characterised in that the dielectric fluid is a silicone oil.

6. A method of filling a housing containing electrical components with a filler as claimed in any one of the preceding claims characterised in that said filler blocks are introduced into spaces within the housing prior to filling the remaining spaces with said slurry.

## Patentansprüche

1. Wärmeleitende Füllmasse zum Einkapseln elektrischer Bauteile, die in einem Gehäuse enthalten sind, wobei die Füllmasse ein Gemisch aus elektrisch isolierenden, thermisch leitenden Partikeln une einem dielektrischen Fluid aufweist, das einen Brei bildet, der vollständig und homogen alle Räume in dem Gehäuse ausfüllt, wobei die Partikel mehr als 50 Vol.-% des Breis vor dem Einführen in das Gehäuse unfassen und dann verdichtbar sind, um eine Paste zu bilden, in welcher die Partikel mehr als 80 Vol.-% einnehmen, dadurch gekennzeichnet, daß die Füllmasse eine Mehrzahl von frei suspendierten Füllmasse-Blöcken aus einem Material enthält, das dieselben Eigenschaften wie dieses Gemisch hat, um das Volumen des Gemisches, das erforderlich ist, um das Gehäuse auszufüllen, zu reduzieren.

2. Wärmeleitende Füllmasse nach Anspruch 1, dadurch gekennzeichnet, daß die Partikel einen mittleren Durchmesser von etwa 150 Micrometer haben.

3. Wärmeleitende Füllmasse nach Anspruch 1 oder 2, dadurch gekennzeichnet, daß die Partikel aus einem keramischen Material gebildet sind.

4. Wärmeleitende Füllmasse nach Anspruch 3, dadurch gekennzeichnet, daß das keramische Material aus der Gruppe ausgewählt ist, welche Metalloxide, Metallnitride und Metallkarbide umfaßt.

5. Wärmeleitende Füllmasse nach einem der Ansprüche 1-4 dadurch gekennzeichnet, daß das dielektrische Fluid ein Silicon-ö1 ist.

6. Verfahren zum Füllen eines Gehäuses, das elektrische Komponenten enthält, mit einer Füllmasse nach einem der vorhergehenden Ansprüche, dadurch gekennzeichnet, daß die Füllmasse-Blöcke in Räume innerhalb des Gehäuses vor dem Füllen der Übrigen Räume mit dem Brei eingebracht werden.

## Revendications

1. Charge thermoconductrice pour capsuler des composants électriques contenus dans un boîtier, la charge comprenant un mélange de particules thermoconductrices électriquement isolantes et d'un fluide diélectrique formant une bouillie appropriée pour remplir complètement et de façon homogène tous les espaces à remplir dans ledit boîter, les particules constituant plus de 509 en volume de la bouillie avant d'être introduites dans le boîter et pouvant être ensuite comprimées pour former une pâte, dans laquelle les particules constituent plus de 80% en volume, caractérisée en ce que la charge comprend plusieurs blocs de charge en suspension libre d'une matière ayant les mêmes propriétés que ledit mélange, de manière à réduire le volume dudit mélange requis pour remplir le boiter.

2. Charge selon la revendication 1, caractérisée en ce que lesdites particules ont un diamètre moyen d'environ 150 micromètres.

3. Charge selon l'une quelconque des revendications 1 ou 2, caractérisée en ce que les particules sont formées d'une matière céramique.

4. Charge selon la revendication 3, caractérisée en ce que la matière céramique est choisi dans le groupe comprenant les oxydes métalliques, les nitrures métalliques et les carbures métalliques.

5. Charge selon l'une quelconque des revendications 1 à 4, caractérisée en ce que le fluide diélectrique est une huile de silicone.

6. Procédé de remplissage d'un boiter contenant des composants électriques à l'aide d'une charge telle que revendiquée dans l'une quelconque des revendications précédentes, caractérisé en ce que ledits blocs de charge sont introduits dans des espaces ménagés dans le boiter, avant le remplissage des espaces restants à l'aide de ladite bouillie.
